

[54] SMOKING MATERIALS

[75] Inventor: Jackie L. White, Pfafftown, N.C.  
[73] Assignee: R. J. Reynolds Tobacco Company,  
Winston-Salem, N.C.  
[22] Filed: Mar. 20, 1975  
[21] Appl. No.: 560,021

[52] U.S. Cl..... 131/2; 131/17 R  
[51] Int. Cl.<sup>2</sup>..... A24B 15/00  
[58] Field of Search..... 131/2, 17, 144, 140 C,  
131/140 P

[56] References Cited

UNITED STATES PATENTS

52,976 3/1866 Dawson ..... 131/2  
3,100,492 8/1963 Schmidt ..... 131/2  
3,106,209 10/1963 Torigian ..... 131/2

FOREIGN PATENTS OR APPLICATIONS

687,507 3/1967 Belgium ..... 131/2

OTHER PUBLICATIONS

"The Chemical Composition of Tobacco and Tobacco Smoke" by Stedman, p. 190; Eastern Utilization Res. & Dev. Div. Res. Service U.S.D.A. Penn. 19118, Reviewed 10/18/67.

Shmuk; vol. 3, "The Chem. & Tech. of Tobacco," pp. 602-603, pub. by Pischempromizdat Moscow, 1953.

"Dang. Prop. of Indust. Mat.," by Sax 3 edit., 1968, Reinhold Book Corp.

Primary Examiner—Robert W. Michell

Assistant Examiner—V. Millin

Attorney, Agent, or Firm—Neuman, Williams,  
Anderson & Olson

[57] ABSTRACT

Puffed triticale is used alone or with tobacco to provide smoking materials.

11 Claims, No Drawings

## SMOKING MATERIALS

This invention relates to novel smoking compositions and to products derived therefrom.

It is a principal object of this invention to provide a composition of matter which is advantageous for use as a smoking material.

It is another object of this invention to provide novel compositions containing tobacco which compositions can be used to form products such as cigarettes, cigars, pipe tobacco and the like.

The present invention involves the discovery that triticale which is in an expanded condition and of relatively low density is eminently suitable for use as a smoking material.

In one embodiment, the invention provides smokable compositions comprising a mixture of tobacco and puffed triticale. The puffed triticale serves as a tobacco extender without significant effect on the organoleptic properties of tobacco products in which it is present. In a second embodiment of the invention, puffed triticale is used alone or with other non-tobacco materials to form smoking materials.

The triticale which is utilized as a smoking material in accordance with this invention is triticale which has been processed to expand its volume and decrease its density whereby it is in an expanded condition supportive of combustion. Triticale is a known hybrid derived by combining wheat (genus *Triticum*) and rye (genus *Secale*). Processing of the triticale to expand its volume involves puffing so as to produce a puffed triticale of relatively low density. In general, the bulk density of the puffed triticale employed herein is not greater than about 0.40 gram per cubic centimeter and preferably not greater than about 0.20 gram per cubic centimeter. The expression "puffed triticale" as used herein means triticale kernels which have been expanded to such extent that the bulk density is not greater than 0.40 gram per cubic centimeter when determined on a 12-mesh sample. For this determination of bulk density the triticale is ground in a suitable mill and sieved to recover the 12-mesh (U.S. Sieve Series) portion thereof with a uniformly packed sample of known volume then being weighed.

The volume expansion of triticale can be accomplished by puffing procedures well known to the art. As is known, puffing of triticale is accomplished by gun puffing which is the release of cereal pieces from a pressurized chamber or oven puffing where the cereal dough pieces are exposed suddenly to high temperatures. The oven method may involve exposure to radiant heat on a belt, tumbling in a heated rotating cylinder, exposure to heated rolls, or extrusion at high pressure and elevated temperature. Puffing of triticale and other similar materials is a well developed art and there exist a number of patents relating to puffing processes and apparatus. Puffing of triticale for use in accordance with this invention can be accomplished using known procedures and apparatus such as described in U.S. Pat. Nos. 3,456,575, 2,701,200, 2,231,387, 3,656,965, 3,703,379, 3,556,802, 3,392,660, 3,201,032, 3,660,110 and 3,682,651. After puffing, the puffed triticale is separated from non-puffed kernels by conventional procedures such as screening, air classification and the like. The size and shape of the puffed triticale which is used to form smoking materials is primarily dependent upon its intended use. It is gener-

ally preferred to grind, or more preferably shred, or otherwise comminute, the puffed triticale to a size and shape approximating that of the tobacco with which it is employed. Thus, when employed with tobacco to form cigarettes, the puffed triticale is cut, sliced or shredded to a size and shape similar to the filler tobacco employed therewith. It is preferred to do likewise when the puffed triticale is used with tobacco to form cigars or pipe smoking compositions.

When used with tobacco, puffed triticale is blended with tobacco and the blend is then processed in conventional manner to form tobacco products. For example, puffed triticale is shredded to a size approximating that of cut filler tobacco with which it is blended in desired proportion. The blend is then processed in conventional cigarette making machines to form cigarettes which can be either of the filter or non-filter type. Additive materials such as flavorants, humectants, ash improvers, combustion modifiers, fillers and the like can be incorporated with the tobacco/puffed triticale blends. Pipe or smoking tobacco products can be readily produced by simply blending the puffed triticale with tobacco and flavorants, if any.

It will be appreciated that the use of puffed triticale with tobacco serves to extend the tobacco or reduce the amount of tobacco employed in a product with a concomitant decrease in the amount of nicotine therein. This is achieved without adverse effect on the taste or aroma of the final product. The amount of the puffed triticale which is blended with tobacco can vary widely up to about 50 percent or more by volume of the tobacco.

According to a second embodiment of the invention, puffed triticale is employed as a tobacco substitute by itself or with other non-tobacco materials to form smoking products such as cigarettes, cigars and pipe smoking products. When so used, it is presently preferred that the puffed triticale simulate tobacco and accordingly appropriate procedures can be employed to provide the puffed triticale in desired size and shape. The burning rate, flavor and other properties of non-tobacco smoking products can be altered by incorporating with the puffed triticale suitable additives such as flavorants, tobacco extracts, nicotine, humectants, ash improving additives, etc. The burning rate of puffed triticale is somewhat faster than most natural tobaccos and accordingly, to decrease the burning rate of non-tobacco smoking products, suitable filler materials or combustion modifiers such as magnesium carbonate, calcium carbonate, potassium carbonate, sodium carbonate, magnesium nitrate, calcium nitrate and the like can be incorporated with the puffed triticale. The materials which are used with the puffed triticale to form smoking products are employed in amounts depending upon the effects desired.

When used with or without tobacco to form smoking materials, the puffed triticale is preferably conditioned to a moisture content of say from 6 to 15 percent at which moisture content the material is well adapted for processing to form smoking products.

The following examples illustrate the advantages of the present invention. In the examples the bulk density of the tobacco extender of this invention was determined by weighing a known volume of the puffed triticale as indicated. However, in all cases the bulk density of the materials is less than 0.40 gram per cubic centimeter when determined on a 12-mesh sample thereof.

## EXAMPLE 1

Bulk density measurements were made on puffed triticale which had been previously stored at 60 percent relative humidity until an equilibrium moisture content of about 8 percent was reached. The puffed triticale was then ground in a Waring blender and sieved. Various particle sizes were collected and the bulk densities thereof were determined by weighing a 50 cubic centimeter volume of uniformly packed material. The packing was accomplished by rapping the bottom of the container frequently during the packing operation so that the particles settled evenly. No external pressure was applied to the mass of particles in making this measurement. The densities of the material retained on various mesh screens are shown in Table I. For comparison purposes, the densities of selected tobacco materials are shown in Table II.

TABLE I

| Material Retained on U.S. Standard Sieve Series | Bulk Density |
|-------------------------------------------------|--------------|
| No. 8                                           | 0.0673 g/cc  |
| No. 12                                          | 0.0579 g/cc  |
| No. 14                                          | 0.0769 g/cc  |
| No. 16                                          | 0.0791 g/cc  |
| No. 20                                          | 0.0842 g/cc  |
| No. 30                                          | 0.0871 g/cc  |

TABLE II

| Sample                                                    | Bulk Density |
|-----------------------------------------------------------|--------------|
| Puffed Flue-Cured Tobacco*                                | 0.07 g/cc    |
| Reconstituted Tobacco                                     | 0.19 g/cc    |
| Commercial cigarette blend without casing or top dressing | 0.11 g/cc    |

\*Puffed in accordance with U.S. Pat. No. 3,524,451

These tests demonstrate that the puffed triticale smoking material is highly expanded and low in bulk density when compared to tobacco commonly used for filling cigarettes.

## EXAMPLE 2

The filling capacity of puffed triticale was determined. The shredded puffed triticale was cut in 32 shreds per inch and was very much like tobacco shreds.

In order to measure the filling capacity of a cigarette filler material, a measuring device is used which is essentially composed of a 100 milliliter graduated cylinder having an internal diameter of about 25 millimeters and a piston having a diameter of about 24 millimeters and weighing about 802.5 grams slidably positioned in the cylinder. A 3-gram sample of the material is placed in the cylinder and the piston positioned on it. The gravitational force exerted by the piston corresponds to a pressure of about 2.3 pounds per square inch. The filling value of the sample is the volume to which the 3-gram sample of the material in the cylinder is compressed after the weight of the piston has acted on it for a period of 3 minutes. This pressure corresponds closely to the pressure normally applied by the wrapping paper to the tobacco in cigarettes. By this procedure the filling capacity of the puffed triticale was found to be 42.4 milliliters per 3-gram sample at a moisture content of 8.30 percent.

## EXAMPLE 3

Cigarettes were prepared from shredded puffed triticale by blending either 20 or 50 percent by volume of the shredded triticale with 80 or 50 percent by volume of a commercial cigarette tobacco. The tobacco-puffed triticale blend was then manufactured into cigarettes using Ecusta Ref. 853 paper. The resulting 65-millimeter tobacco rods were combined with 20 millimeters of a 3.3/39,000 cellulose acetate filter and the finished filter cigarettes were smoked under standard FTC conditions to give the following results:

| 15                               | Rod Composition<br>(Rod length: 65 mm) | Rod Weight<br>in grams | TPM*<br>(mg.) | Nicotine<br>(mg.) | FTC**<br>Tar (mg.) |
|----------------------------------|----------------------------------------|------------------------|---------------|-------------------|--------------------|
| All Tobacco                      |                                        | 0.89                   | 23.4          | 1.29              | 17.7               |
| 20% (vol.)<br>Puffed Triticale ] |                                        | 0.77                   | 21.7          | 1.09              | 16.8               |
| 80% (vol.) Tobacco ]             |                                        |                        |               |                   |                    |
| 50% (vol.)<br>Puffed Triticale ] |                                        | 0.59                   | 20.2          | 0.76              | 15.2               |
| 50% (vol.)<br>Tobacco ]          |                                        |                        |               |                   |                    |

\*Total Particulate Matter

\*\*As determined by standard procedures of Federal Trade Commission.

Cigarettes containing 20 percent by volume of the shredded puffed triticale were smoked by expert panelists in comparison with an all tobacco control cigarette. Forty-five percent of the panelists indicated either a preference for the triticale-containing cigarette or no difference between the test and control cigarettes as far as preference was concerned. Thirty-five percent of the panelists declared that the test cigarette was milder while 25 percent detected no difference in mildness. Better over-all flavor was attributed to the test cigarettes by 30 percent of the panelists.

The use of puffed triticale with tobacco to produce useful products possesses numerous advantages. Thus, use thereof permits a significant reduction in the utilization of tobacco. Not only is the use of less tobacco in a tobacco product obviously advantageous from an economic standpoint, but the reduction of nicotine in such products may be highly desirable. The reduction of so-called "tars" may also be realized through the use of puffed triticale in smoking products since particulate matter produced per unit volume of puffed triticale is substantially less than that for tobacco due to the significantly lower density of puffed triticale. The nicotine-free puffed triticale, when blended with tobacco, does not cause adverse effects on the quality of the final product. The puffed triticale is easily processed, readily available at relatively low cost and does not detract from the taste or aroma of the tobacco product. The puffed triticale is non-friable in nature, does not collapse as a cigarette is smoked nor does it hinder combustion or puffing of cigarettes in which it is employed.

Those modifications and equivalents which fall within the spirit of the invention are to be considered a part thereof.

What is claimed is:

1. A smoking material which contains comminuted puffed triticale in a form resembling cut cigarette filler tobacco or cut pipe tobacco.
2. A smoking material in accordance with claim 1 wherein the puffed triticale is in the form of shreds.
3. A smoking material in accordance with claim 1 which also contains tobacco.

5

4. A smoking material in accordance with claim 3 wherein the puffed triticale is employed in an amount up to 50 percent by volume of the tobacco.

5. A cigarette whose filler contains comminuted puffed triticale in a form resembling cut cigarette filler tobacco.

6. A cigarette in accordance with claim 5 wherein the puffed triticale is in the form of shreds.

7. A cigarette in accordance with claim 5 whose filler also contains tobacco.

6

8. A cigarette in accordance with claim 7 wherein the puffed triticale is employed in an amount of up to 50 percent by volume of the tobacco.

9. A process of preparing a cigarette which comprises wrapping with a cigarette paper a filler material containing comminuted puffed triticale in a form resembling cut cigarette filler tobacco.

10. A process in accordance with claim 9 wherein the puffed triticale is in the form of shreds.

11. A process in accordance with claim 9 wherein said filler material also contains tobacco.

\* \* \* \* \*

15

20

25

30

35

40

45

50

55

60

65